# EUROPEAN PATENT SPECIFICATION

(11) **EP 0 549 496 B1**
(45) Date of publication and mention of the grant of the patent: **08.04.1998**
(21) Application number: 92420480.3
(22) Date of filing: 23.12.1992
(51) Int. Cl.: G03C 1/38

(54) **Glycoside surfactants as coating aids for photographic layers**
Glycosidische Tenside als Überzugsmittel für fotografische Schichten
Tensio-actifs glycosidiques utilisés comme agents de revêtement pour couches photographiques

(30) Priority: 24.12.1991 US 812928
(43) Date of publication of application: 30.06.1993
(73) Proprietor: EASTMAN KODAK COMPANY, Rochester, New York 14650-2201 (US)
(72) Inventor: Orem, Michael William, c/o EASTMAN KODAK COMPANY, Rochester, New York 14650-2201 (US)
(74) Representative: Parent, Yves

(56) References cited:
- US-A- 3 507 660
- US-A- 4 675 127
- PATENT ABSTRACTS OF JAPAN vol. 4, no. 149 (P-032)21 October 1980
- PATENT ABSTRACTS OF JAPAN vol. 16, no. 323 (P-1386)15 July 1992

## Description

This invention relates to surfactants as coating aids for gelatin coating solutions, particularly to such solutions used for photographic purposes. This invention also relates to the use of long chain alkyl glycosides as coating aid surfactants for such solutions.

In the preparation of a photographic material, it is usual to coat a support with one or more layers comprising an aqueous solution of a hydrophilic colloid binder, e.g. gelatin. Such layers include, for example, silver halide emulsion layers, intermediate layers, antihalation layers, filter layers, antistatic layers and protective layers. For multilayer materials, the layers may be coated simultaneously on conventional photographic supports as described in U.S. Pat. Nos. 2,761,791 and 3,508,947.

There are two primary methods for coating photographic materials. One is the bead coating process; see U.S. 2,681,294, 2,761,417, and 4,525,392. These references illustrate applying multiple layers of photographic materials using the bead coating method, and also illustrate apparatus for carrying out the method. The second primary method is the curtain coating process. U.S. 3,632,372 and 4,569,863 illustrate coating and apparatus for conducting the Process.

In producing the thin hydrophilic colloid layers of such photographic materials, it is required that coating solutions be coated uniformly without the formation of repellency spots or craters, also referred to as repellencies. A repellency is a round, oval-shaped or comet-shaped indentation or crater, or a vestige of such a disturbance which has partially healed after formation. Imperfections of this type are present in the layer being coated, if one layer is coated, or in one or more layers, if more of than one layer is coated simultaneously. Repellencies are formed during the coating process, or shortly thereafter, that is, when the solution of gelatin (or other hydrophilic colloid) in the coating is still fluid or mobile. Repellencies are usually produced by the presence of small particles or droplets of insoluble materials in the form of addenda, impurities or contaminants which are (i) in contact with the uppermost liquid-air interface of the coated layer(s) and (ii) have surface activity, that is, they are capable of reducing the surface tension of the liquid-air interface in isolated areas during the coating process.

Solutions coated in the preparation of photographic materials often contain dispersed, insoluble photographic addenda, which might include organic solvents, or addenda to alter certain physical properties, which might include lubricants and impurities in the lubricants, each of which may be capable of imparting repellencies to the coated layer(s). Even photographic gelatin may contain insoluble residues of naturally-occurring animal fats and fatty acids which are capable of imparting repellencies to the coated layer(s). Also, surface active contaminants may originate from external sources during the preparation of the coating composition or during coating. For example, the layer(s) being coated, or immediately after coating, may be unintentionally showered by droplets of lubricating oils used in the apparatus.

In the application of gelatin coating compositions to a support such as film base or paper, it is desirable to have a coating aid surfactant present in the coating composition, in order to facilitate application of the coating to the surface being coated. In this context, the compound or compounds used as coating aid surfactants in this invention are compounds which are effective in reducing the surface tension of the gelatin-containing coating composition. The presence of a coating aid surfactant, in the coating or coatings, assists in obtaining layers which, when dry, are of uniform or substantially uniform thickness,and are free, or substantially free, of imperfections such as repellencies.

Over the years, many compositions have been suggested for use as coating aids. In this regard, reference is made to section XI of Research Disclosure, Issue **308**, (December 1989), pp.993-1015. However there are relatively few water soluble surfactants that have achieved wide spread use as coating aids, since many surfactants of this type are not very effective in controlling imperfections such as repellencies, or have undesirable photographic properties, and very few of these preferred surfactants have nonionic structures.

One category of nonionic saccharidic coating aid surfactants described in the prior art comprises long-chain alkyl ethers, esters, and urethane of sucrose, where sucrose is the hydrophilic group of the surfactant molecule. In U.S. 3,507,660, Nishio, et al. describe long-chain alkyl ethers and urethanes of sucrose as coating aid surfactants of photographic materials. In U.S. 3,516,833, Haage, et al. describe long-chain alkyl esters of sucrose as coating aid surfactants. In U.S. 3,220,847, Knox describes the half esters of sucrose and alkyl succinic acids as coating aid surfactants, and in U.S. 3,564,576, Knox describes long chain alkyl esters of sucrose in combination with sodium maleopimarate as mixtures of surfactants with good coating aid properties.

Sugar surfactants are among the materials taught as useful with compositions comprising couplers in a fine state of subdivision; U.S. 5,013,640.

The use of these prior art compositions as coating aids has been limited by their limited water solubility, by their limited solubility in gelatin containing solutions, or by their limited ability to minimize repellency formation.

Thus a need exists for a new nonionic surfactant having increased solubility properties in gelatin/water solutions over the prior art materials.

This invention provides a composition of matter comprising (i) gelatin in water, said composition comprising from 2.5 to 20 weight percent gelatin based on gelatin in water and, (ii) from 0.05 to 0.30 weight percent based on the solution weight of a coating aid surfactant, a glycoside having the formula

CₙH₂ₙ₊₁ -O-(C₆H₁₀O₅)_{X} -H, (I)

wherein the group within the parentheses represents a unit of glucose, n represents mean values of 9, up to 16, and x is a distribution with a mean value greater than 1 and less than 2, and (iii) an auxiliary anionic or nonionic surfactant in sufficient amount to completely dissolve or substantially completely dissolve the glycoside in the composition.

In a highly preferred embodiment, the above composition provides a top layer of a simultaneously coated multilayer pack of a photographic material coated by bead coating methods. In another embodiment, the above composition provides a top layer and/or a bottom layer of a simultaneously coated multilayer pack of a photographic material coated by curtain coating methods. For the purpose of this invention, a "top" layer of a simultaneously coated multilayer pack, that is, a pack of two or more layers coated together, is defined as the layer farthest from the web. Similarly, the "bottom" layer of a simultaneously coated multilayer pack is defined as the layer closest to the web. The term "web" refers to a continuous length of prepared film base or paper base and can include previously coated and dried layers, such as emulsion layers or antihalation layers. In another embodiment, the above composition provides a single layer, coated alone, of a photographic material.

In the embodiments described in the paragraph immediately above, the layer having the coating aid surfactant of formula (I) may also contain a silver halide and/or other image forming material, or, alternatively, it may not contain image forming materials. The layer formed from the above composition can be a protective overcoat layer of one or more image forming layers coated on one or both sides of the web, for example, either a color or black-and-white film or paper product. Alternatively, the layer formed from the above composition can be a protective overcoat layer of a pelloid backing coating of a color or black-and-white film product. An overcoat layer may contain other ingredients commonly present in such layers, and known in the art. Alternatively, the layer formed from the above composition can be a layer other than the overcoat layer of a multilayer color photographic material, such as a nonimage forming layer located between image forming layers, resulting from the stepwise application of two or more separate multilayer packs in the process of manufacturing a photographic material with a large number of individual layers.

The glycoside surfactants employed in this invention are useful as coating aids in such gelatin-containing layers for photographic materials, because they confer improved thickness uniformity, i.e., fewer repellency spot imperfections in the layers. The present invention provides alternative aqueous gelatin compositions to that of the prior art, showing at least equivalent coating propeties.

This is a substantial improvement in the art. Glycoside surfactants of the type employed in this invention are readily available; hence this invention is readily adaptable by industry.

In this invention the glycoside surfactants are used as coating aid surfactants which are effective in reducing the surface tensions of gelatin-containing coating compositions. The reduction in the surface tension of gelatin solution by the addition of the glycoside surfactants can be demonstrated by laboratory measurements of surface tensions using the Wilhelmy plate technique. The surface tension of a solution of nondeionized, lime derived bone gelatin (70 grams per liter) in a glass beaker at a temperature of 110°F (43°C) is 40-42 dynes/cm, and after adding glycoside surfactant APG 325 at 1.0 gram per liter is 28 dynes/cm.

This invention provides a composition comprising from 2.5 weight percent to 20 weight percent of gelatin in water and from 0.05 to 0.30 of the coating aid surfactant having formula (I) as above described, and preferably from about 5 to about 12 weight percent gelatin in water, and from about 0.05 to about 0.3 weight percent of the coating aid surfactant. Thus, the compositions of this invention provide one or more layers of a photographic material.

In another preferred aspect, this invention provides a photographic material, e.g. a film or paper, having at least one layer comprising a dried layer formed from a coat or melt having the above composition.

This invention can be used with any gelatin that is employed in photographic products, including bovine bone gelatin derived by treatment with base, e.g. lime. However, the invention is not limited to such a gelatin. In this regard, the utility of the invention is demonstrated below in a composition based on acid derived porcine skin gelatin. This type of gelatin generally gives rise to a more frequent occurrence of repellencies than the above-mentioned bovine gelatin.

The gelatin in the compositions of this invention can optionally be hardened by any hardener that is known in the art. Hardeners and their use are described in Section X of Research Disclosure, *supra.* It is to be understood that the presence or absence of a hardener is not a critical feature of this invention.

The compositions of this invention comprise gelatin in water. Typically the gelatin concentration in a coating composition to be applied to paper or a film-base support is from about 2.5 to about 20 weight percent gelatin. Top layer coating compositions of this invention preferably have from about 5 to about 12 weight percent gelatin.

In addition to hardeners and/or the reaction product of the gelatin and the hardener, the compositions of this invention may contain other photographic chemicals of the usual types found in photographic layers. For example, the top layers within one of the preferred embodiments of this invention may contain antistatic agents, matting agents, plasticizers, lubricants, and other materials that are not involved in image formation. For examples of matting agents, see Section XVI of the Research Disclosure, *supra,* for antistatic materials, Section XIII, and pasticizers and lubricants, Section XII.

The range of concentration within which the coating aid is used depends on the source of repellency. It also depends on whether other surface active agents in addition to the auxiliary surfactant are present.

Preferred glycosides for use in this invention, and within the above general formula, are manufactured by the Henkel Corporation and sold as APG Glycosides. Such glycosides are described in Henkel technical bulletins. Preferred APG Glycosides are APG 225, APG 300, and APG 325 Glycosides.
The glycoside coating aid surfactants is used with an auxiliary surfactant to increase the solubility of the glycoside surfactant in the composition. Thus for example, in compositions in which gelatin is the hydrophilic colloid the glycoside is admixed with an auxiliary nonionic or anionic surfactant. Example of such auxiliary surfactants are nonionic long-chain alkyl (6-18 carbons) aryl polyglycidol (5-20) ethers, and representative anionic surfactants are alkyl sulfates, alkyl sulfonates, alkyl aryl sulfonates, alkyl polyethoxy sulfates, alkyl aryl polyethoxy sulfates, and alkyl aryl polyethoxy sulfonates, containing 6-18 carbons in their alkyl groups.

In general, the amount of the auxiliary surfactant is about 25 to 200 percent by weight based on the weight of the glycoside coating aid surfactant.

Photographic elements according to the invention generally comprise at least one light-sensitive layer, such as a silver halide emulsion layer. This layer may be sensitized to a particular spectrum of radiation with, for example, a sensitizing dye, as is known in the art. Additional light-sensitive layers may be sensitized to other portions of the spectrum. The light-sensitive layers may contain or have associated therewith dye-forming compounds or couplers. For example, a red-sensitive emulsion would generally have a cyan coupler associated therewith, a green-sensitive emulsion would be associated with a magenta coupler, and a blue-sensitive emulsion would be associated with a yellow coupler. Other layers and addenda, such as antistatic compositions, subbing layers, surfactants, filter dyes, protective layers, barrier layers, development inhibiting releasing compounds, and the like can be present in photographic elements of the invention, as is well-known in the art. Detailed description of photographic elements and their various layers and addenda can be found in *Research Disclosure* 17643 Infra, and in James, *The Theory of the Phonographic Process*, 4th, 1977.

The gelatin-containing layer of this and other layers in the element may be coated by any of the known coating methods, such as curtain coating, roller coating, bead coating, doctor blade coating, dip and air knife coating, and the like. The layer is generally dried by simple evaporation, which may be accelerated by known techniques such as convection heating. Known coating and drying methods are described in more detail *Research Disclosure* 17643, December, 1978. To demonstrate the advantage of the coating aids of this invention over prior art surfactants, coatings of gelatin solutions were made on a narrow width coating machine and the coatings were visually examined for comparisons of uniformity of layer thicknesses. For the purposes of the following example, a variety of gelatin which has a high propensity for forming repellency spots was used in the top layer. Coatings made without any coating aid surfactant in the top layer had a large number of repellency spots, and repellency spots were also observed in coatings containing APG 300 or 325 alone or the comparison compound sucrose laurate alone in the top layer solution. But when the mixtures of APG 300 or 325 and nonionic auxiliary surfactant were added to the top layer, the resulting coatings had fewer repellency spots than the coatings made with sucrose laurate alone or combined with the nonionic auxiliary surfactant or with sodium maleopimerate. Experimental details are set forth below.

### Example 1

A simultaneous 3-layer coating was made with a conventional, multi-slide, bead coating hopper onto subbed polyester film support at a coating speed of 90 meters per minute. A solution of acid-derived photographic grade pigskin gelatin (100 grams per liter of solution) was prepared for the top layer. The middle layer consisted of a solution of lime-derived bone gelatin to which dispersed carbon particles were also added to provide an optical density in the middle layer of about 1.0, to allow the observation of layer thickness uniformity by visual examination. The bottom layer consisted of a solution of lime-processed bone gelatin without any carbon added. Repellency spots forming in the top layer during the coating process also disturbed the middle layer (containing the carbon) and were observed by visual inspection and counted according to number and size per unit area. Spots were counted in two categories, large enough to see without magnification and small enough that 7x magnification was required. The results comparing various surfactants are shown in Table I. Without surfactant in the top layer solution, the coatings had a large number of repellency spots in both size categories. Coatings made with APG 300 (0.1 percent) or APG 325 (0.1 percent) alone or with the comparison compound sucrose laurate (0.1 percent) alone in the top layer solution also had large numbers of repellency spots. Although the numbers of repellency spots were much lower in coatings containing 0.1 or 0.2 percent of Surfactant 10G (used in other coatings as an auxiliary surfactant) alone, the coatings containing the fewest repellency spots of all the conditions shown were those containing mixtures of APG 300 (0.1 percent) and Surfactant 10G (0.08 or 0.16 percent) as an auxiliary surfactant or mixtures of APG 325 (0.1 percent) and Surfactant 10G (0.08 or 0.16 percent) as an auxiliary surfactant. The mixtures of the glycoside coating aid surfactants of this invention and a nonionic auxiliary surfactant were much more effective in preventing the formation of repellency spots in coating than the representative prior art surfactant alone or in mixtures with sodium maleopimarate or with Surfactant 10G.

Materials used in this example are described as follows:
(C) Sucrose monolaurate, representative comparison compound (prior art, U.S. 3,516.833); material used was GRILLOTEN LSE 65, R.I.T.A. Corporation, P.O. Box 585, Woodstock, IL, 60098.
(A1) APG 300 glycoside compound where n = mixture of 9, 10, and 11, and $\overline{\text{x}}$ ≃ 1.4 in formula (I) (Henkel product literature).
(A2) APG 325 glycoside compound where n = mixture of 9, 10, and 11, and $\overline{\text{x}}$ ≃ 1.6 in formula (I) (Henkel product literature).
(B1) Surfactant 10G from Olin Corporation is a mixture of nonyl phenoxy polyglycidol (5-14) ethers.
(B2) Sodium maleopimarate (used in mixture in the prior art, U.S. 3,564,576) is a compound prepared by reacting maleic anhydride with pimaric acid and neutralizing with sodium hydroxide.

**TABLE I**

| Surfactant (first)¹ | | Surfactant (second)¹ | | Repellency spots number observed | |
|---|---|---|---|---|---|
| compound | conc. wt. % | compound | conc. wt. % | w/o mag² | magnified 7x³ |
| none | --- | none | --- | 220 | 1800 |
| A1 | 0.1, 0.2 | none | --- | VH⁴ | VH |
| A2 | 0.1, 0.2 | none | --- | VH | VH |
| C | 0.1, 0.2 | none | -- | VH | VH |
| B1 | 0.1 | none | --- | 19 | 600 |
| B1 | 0.2 | none | --- | 10 | 700 |
| A1 | 0.1 | B1 | 0.08 | 8 | 3 |
| A1 | 0.1 | B1 | 0.16 | 0 | 6 |
| A2 | 0.1 | B1 | 0.08 | 0 | 11 |
| A2 | 0.1 | B1 | 0.16 | 1 | 21 |
| C | 0.1 | B1 | 0.05 | VH | VH |
| C | 0.1 | B1 | 0.12 | 7000 | VH |
| C | 0.1 | B1 | 0.22 | 9000 | VH |
| C | 0.1 | B2 | 0.1 | 1800 | 1900 |
| C | 0.1 | B2 | 0.2 | 1100 | 760 |

| | | | | | |
|---|---|---|---|---|---|
| key: 1 in top layer solution, wt. % based on solution wt. | | | | | |
| 2 in area 0.46 m² of coating | | | | | |
| 3 in area 310 cm² of coating | | | | | |
| 4 VH = very high number | | | | | |

## Claims

1. A composition characterized in that it comprises (i) gelatin in water, said composition comprising from 2.5 to 20 weight percent gelatin, based on gelatin in water, (ii) from 0.05 to 0.30 weight percent, based on the solution weight, of a coating aid surfactant having the formula:
CₙH₂ₙ₊₁-O-(C₆H₁₀O₅)ₓ-H
wherein C₆H₁₀O₅ represents a glucose unit, n represents mean values of 9 to 16, and x is a distribution with mean values greater than 1 and less than two, and (iii) an auxiliary nonionic or anionic surfactant in an amount sufficient to dissolve completely said coating aid surfactant in said composition.

2. A composition of Claim 1 characterized in that the amount of said auxiliary surfactant is from 25 to 200 percent by weight based on the weight of said coating aid surfactant.

3. A photographic material characterized by a support having thereon at least one layer comprising a dried coating composition of Claim 1.

4. A method for preparation of a photographic material, said method characterized by coating a layer having the composition of Claim 1.

## Patentansprüche

1. Zusammensetzung, dadurch gekennzeichnet, daß sie aufweist (i) Gelatine in Wasser, wobei die Zusammensetzung 2,5 bis 20 Gew.-% Gelatine, bezogen auf Gelatine in Wasser, enthält, (ii) 0,05 bis 0,30 Gew.-%, bezogen auf das Lösungsgewicht an einem oberflächenaktiven Mittel als Beschichtungshilfe mit der Formel:
CₙH₂ₙ₊₁-O-(C₆H₁₀O₅)ₓ-H
worin C₆H₁₀O₅ eine Glukoseeinheit darstellt, n für Mittelwerte von 9 bis 16 steht und x eine Verteilung mit Mittelwerten von größer als 1 und kleiner als 2 ist, und (iii) ein nichtionogenes oder anionisches oberflächenaktives Hilfsmittel in einer Menge, die ausreicht, um das als Beschichtungshilfe verwendete oberflächenaktive Mittel in der Zusammensetzung vollständig zu lösen.

2. Zusammensetzung nach Anspruch 1, dadurch gekennzeichnet, daß die Menge an dem oberflächenaktiven Hilfsmittel bei 25 bis 200 Gew.-%, bezogen auf das Gewicht des als Beschichtungshilfe verwendeten oberflächenaktiven Mittels liegt.

3. Photographisches Material, gekennzeichnet durch einen Träger, auf dem sich mindestens eine Schicht befindet mit einer getrockneten Beschichtungszusammensetzung nach Anspruch 1.

4. Verfahren zur Herstellung eines photographischen Materials, gekennzeichnet duch Auftragen einer Schicht mit der Zusammensetzung nach Anspruch 1.

## Revendications

1. Composition caractérisée en ce qu'elle comprend (i) de la gélatine dans de l'eau, ladite composition comprenant de 2,5 à 20 % en poids de gélatine, par rapport au poids de la gélatine dans l'eau, (ii) de 0,05 à 0,30 % en poids, par rapport au poids de la solution, d'un agent tensioactif utilisé comme adjuvant de couchage représenté par la formule :
CₙH₂ₙ₊₁-O-(C₆H₁₀O₅)ₓ-H
où C₆H₁₀O₅ représente un motif glucose, n représente les valeurs moyennes de 9 à 16 et x est une répartition avec des valeurs moyennes supérieures à 1 et inférieures à 2 et (iii) un agent tensioactif anionique ou non ionique auxiliaire en quantité suffisante pour dissoudre totalement ledit agent tensioactif utilisé comme adjuvant de couchage dans ladite composition.

2. Composition selon la revendication 1, caractérisée en ce que la quantité dudit agent tensioactif auxiliaire est comprise entre 25 et 200 % en poids par rapport au poids dudit agent tensioactif utilisé comme adjuvant de couchage.

3. Produit photographique caractérisé par un support recouvert d'au moins une couche comprenant la composition de couchage de la revendication 1, séchée.

4. Procédé de préparation d'un produit photographique, ledit procédé étant caractérisé en ce que l'on applique une couche ayant la composition indiquée dans la revendication 1.
